

# UNITED STATES PATENT OFFICE.

FRANK D. CARNEY, OF STEELTON, PENNSYLVANIA, ASSIGNOR TO THE PENNSYLVANIA STEEL COMPANY, OF STEELTON, PENNSYLVANIA, A CORPORATION OF PENNSYLVANIA.

## PROCESS FOR MANUFACTURING STEEL FROM CHROMIFEROUS PIG-IRON.

No. 902,052.

Specification of Letters Patent.

Patented Oct. 27, 1908.

Application filed August 28, 1907. Serial No. 390,476.

*To all whom it may concern:*

Be it known that I, FRANK D. CARNEY, a citizen of the United States, residing at Steelton, county of Dauphin and State of Pennsylvania, have invented a new and useful process for Manufacturing Steel from Chromiferous Pig-Iron, of which the following is a specification.

I have discovered, after many experiments, that pig iron rich in chromium, produced from chromiferous ores, as a starting metal, when treated in a pneumatic converter at a comparatively low temperature, that is a temperature that does not reach a point at which it will reduce the products of the oxidation of the chromium and cause metallic chromium to reenter the metal, can successfully be converted into useful steel.

In carrying out my process having produced from chromiferous ores in the blast furnace, pig iron preferably with a low content of silicon, I charge the same in a melted state into a Bessemer or other pneumatic converter.

The pig iron with which I have had experience in carrying out my process varies in its composition, and contains as elements of interest to state, of chromium from 2% to 40%; of silicon from 0.50% to 2.00%; of manganese 0.50% to 0.80%; of phosphorus 0.15%; and of total carbon in the neighborhood of 4.50%.

The oxidation of the silicon develops heat, as is well known, early in the blow, and I have found that the oxidation of the chromium, likewise develops much heat, being about one-half that developed by the oxidation of silicon, such heat being developed at about the same time as that from the oxidation of the silicon, and I rely upon such heat so developed as an important part of the heat necessary to maintain the proper fluidity of the metal.

The blowing operation should be carefully conducted, the temperature being so controlled as not to accelerate rapidly. The temperature should be maintained comparatively low during the blow, that is, so that as far as practicable it will not reach a point at which the products of oxidation of the chromium will be reduced and metallic chromium be caused to reenter the metal. This I do in the earlier part of the blow, by prefer-

ably prior to charging the melted chromiferous iron into the converter (although this may be done after the commencement of the blow) putting in the converter cold steel scrap or pig iron determined by weight in proportion to the chromium and silicon content of the chromiferous pig iron, so that some of the excess of heat that results from the oxidation by these elements oxidized in the earlier part of the blow, may be absorbed by the melting of such cold metal; and during the blow I add further cold metal or admit watery vapor or steam into the blast, or use any other cooling methods to maintain such comparatively low temperature, during the blow, which terminates when the usual elimination of the carbon has been effected.

The result of the maintenance of a proper low temperature, will be the retention, in the slag of the products of the oxidation of the chromium.

As one way of indicating the proper temperature to be maintained, I would say that the temperature should be kept as low as possible throughout the blow, without incurring risk of skulling the teeming ladle or closing the nozzle thereof, as teeming is usually practiced in Bessemer plants.

Analysis of the metal at the end of the blow will show that the greater part of the chromium has been eliminated, and for some purposes this metal preferably after being separated from the slag, may be finished by the addition of the usual rebarburizing agents for the production of commercial steel having a small content of chromium.

In carrying out my process I may use a pneumatic converter with the usual "acid" lining, or a pneumatic converter with the usual "basic" lining (employing with the latter loose basic material such as lime), with similar results so far as the substantial elimination of the chromium is concerned.

It may be desirable in some cases, where, as an example, chromiferous pig iron, such as that with which I have had experience before mentioned, contains 0.15 per cent. of phosphorus, and silicon preferably below 1.25 per cent., to use a pneumatic converter with a "basic" lining, whereby fifty-five to seventy-five per cent. of such phosphorus can be eliminated without the usual "after blow" of the ordinary basic Bessemer proc-

ess, the heat from the oxidation of the chromium enabling this to be done.

In carrying out my process in such a converter a large proportion of the chromium is eliminated and reduction of phosphorus as aforesaid is effected to a content consistent with many uses of steel, and the resulting metal after being preferably separated from the slag may be subjected to re-carburization and teemed for further manipulation. I prefer, however, to use a pneumatic "acid" lined converter, when the chromiferous pig iron, such as that with which I have had experience before mentioned, contains about 0.50 per cent. and upwards of silicon, on account of the cost per heat blown being less than when using a "basic" lined pneumatic converter, and the heat conditions being under better control.

For many purposes it is desirable or necessary to further treat the metal which has been subjected to my process in either kind of pneumatic converter, for the elimination of phosphorus and any small percentage of chromium. This, if the metal has been treated in an acid lined pneumatic converter, is done by transferring the blown metal into a basic lined open hearth furnace into which I have charged a comparatively small quantity of usual basic slag forming material that is heated up prior to charging the said metal. I also charge into said furnace a comparatively small quantity of pig iron either cold or in a molten state. This serves to furnish the carbon and other oxidizable elements requisite to produce the customary "boil". The process then proceeds for the elimination of the phosphorus and any small percentage of chromium quickly, the time being from about one to three hours, depending upon the size of the furnace. The slags formed in this process give no trouble whatever.

If the product is desired for a steel containing over 0.30% carbon and upward, for rails, springs and the like, I preferably add at the end of the basic open hearth treatment a quantity of molten pig iron, free from chromium and having a low content 50 of phosphorus, preferably not exceeding 0.15% with or without other recarburizing agents containing manganese. If the product is to be a low carbon steel containing below 0.30% carbon, I do not add pig iron as 55 above mentioned, but finish the metal with recarburizing agents after the metal has been tapped into the ladle.

If the metal has been treated in a pneumatic converter with a basic lining, it can be further treated for the elimination of any small percentage of chromium remaining therein by transferring it into an acid lined open hearth furnace, and then subjecting it to the same process as that just described 65 with reference to its treatment in a basic

lined open hearth furnace, with the exception that no basic slag forming material is used.

As a specific example, the following are the results obtained with 24,000 lbs. of chromiferous pig iron charged in a molten state into an acid Bessemer converter. This metal contained silicon 1.44%; chromium 3.41%; phosphorus 0.10% and carbon 4.50%. The scrap added in the converter to reduce the temperature was 5,000 lbs. and the heat was blown twenty-two minutes, using steam in blast 15 minutes to keep down the temperature. The result was—metal containing 0.36% chromium, 0.04% silicon, 0.091% phosphorus and 0.03% carbon. The Bessemer slag analyzed—38.97% FeO, 28.48% SiO<sub>2</sub>, 31.11% Cr<sub>2</sub>O<sub>3</sub>; and 4.08% MnO. 25,000 lbs. of the blown Bessemer metal just mentioned was transferred to an eighteen ton basic open hearth furnace containing 2,000 lbs. of cold chromiferous pig iron, 600 lbs. lime, 250 lbs. mill scale and 200 lbs. fluor-spar. Seventy-eight minutes after the blown Bessemer metal was charged, 4,500 lbs. of molten hematite iron was added for recarburizing and six minutes later the heat was tapped into a ladle containing 350 lbs. ferro-manganese and 100 lbs. ferro-silicon. The total time in open-hearth furnace was one hour and twenty-four minutes. The weight of the finished metal was 31,900 lbs. The finished metal analyzed—carbon 0.516, chromium 0.24; manganese 0.92; phosphorus 0.024; silicon 0.05; sulfur 0.07.

I claim as my invention, and desire Letters Patent, viz:

1. The process of manufacturing steel which consists in blowing chromiferous pig iron in a pneumatic converter, and maintaining a comparatively low temperature during the progress of the blow, substantially as described.

2. The process of manufacturing steel which consists in blowing chromiferous pig iron having a low content of silicon in a pneumatic converter, and maintaining a comparatively low temperature during the progress of the blow substantially as described.

3. The process of manufacturing steel which consists in blowing chromiferous pig iron in a pneumatic acid converter, and maintaining a comparatively low temperature during the progress of the blow substantially as described.

4. The process of manufacturing steel which consists in blowing chromiferous pig iron having a low content of silicon in a pneumatic acid converter, and maintaining a comparatively low temperature during the progress of the blow, substantially as described.

5. The process of manufacturing steel which consists in blowing chromiferous pig iron in a pneumatic converter, and main-

taining a comparatively low temperature during the progress of the blow by cooling methods substantially as described.

6. The method of manufacturing steel which consists in blowing a chromiferous pig iron in a pneumatic converter, at a comparatively low temperature, obtained largely by melting of scrap charged in the converter before beginning the blow, for absorbing excess 10 of heat derived from oxidation of chromium and silicon, substantially as described.

7. The process of making steel which comprises blowing chromiferous pig iron in a pneumatic converter maintaining a comparatively low temperature during the progress of the blow, separating metal and slag and charging such blown metal into an open hearth furnace with sufficient pig iron to produce the boil and then adding pig iron free 20 from chromium, substantially as described.

8. The process of making steel which comprises blowing chromiferous pig iron in an acid pneumatic converter separating metal and slag and charging such blown metal into 25 an open hearth furnace with sufficient melted pig iron to produce the boil and then adding pig iron free from chromium, substantially as described.

9. The process of making steel which comprises blowing chromiferous pig iron in a pneumatic converter, separating metal and slag and charging such blown metal into an open hearth furnace with sufficient pig iron to produce the boil and then adding an iron 30 addition of high carbon low phosphorus pig 35 iron free from chromium, substantially as described.

10. The process of making steel which comprises blowing chromiferous pig iron in a pneumatic converter, separating metal and 40 slag and charging such blown metal containing less than .60% of chromium into an open hearth furnace with sufficient pig iron to produce the boil and then adding pig iron free 45 from chromium, substantially as described.

11. The process of making steel which comprises blowing chromiferous pig iron in a pneumatic converter, separating metal and slag and charging such blown metal containing less than .60% of chromium into a basic 50 open hearth furnace with sufficient melted pig iron to produce the boil to thereby heat up the bath and remove a small per centage of chromium and the phosphorus, and then 55 adding an iron addition of high carbon low phosphorus pig iron free from chromium, substantially as described.

12. The process of making steel which

comprises blowing chromiferous pig iron in a pneumatic converter, separating metal and 60 slag and charging such blown metal containing less than .60% of chromium into a basic open hearth furnace with sufficient cold pig iron to produce the boil to thereby heat up the bath and remove a small per centage 65 of chromium and the phosphorus and then adding, just before tapping, an iron addition of high carbon low phosphorus pig iron free from chromium and containing manganese, substantially as described. 70

13. The process of making steel which comprises blowing chromiferous pig metal in a pneumatic converter, separating metal and slag and charging such metal into an open hearth furnace with sufficient chromiferous 75 pig metal to produce a boil and adding heat to the bath by the oxidation of the chromium in the pig metal, substantially as described.

14. The process of making steel which 80 comprises blowing chromiferous pig metal in a pneumatic converter, separating metal and slag and charging such metal into an open-hearth furnace with sufficient chromiferous pig metal to produce a boil and adding heat 85 to the bath by the oxidation of the chromium in the pig metal, then partly recarbonizing by the addition of the usual high carbon low phosphorus pig metal free from chromium and finishing the steel, substantially as 90 described.

15. The process of making steel which comprises blowing chromiferous pig metal in a pneumatic converter separating metal and slag and charging such metal into an open hearth furnace with sufficient chromiferous 95 pig metal to produce a boil and adding heat to the bath by the oxidation of the chromium in the pig metal and finishing the metal, substantially as described. 100

16. The process of making steel, which comprises blowing chromiferous pig iron in a pneumatic converter, maintaining a comparatively low temperature during the progress of the blow, separating metal and slag, 105 and charging such blown metal into an open-hearth furnace with sufficient pig iron to produce the boil, substantially as described.

In testimony that I claim the foregoing as my invention, I have signed my name in 110 presence of two subscribing witnesses.

FRANK D. CARNEY.

Witnesses:

M. B. PHILIPP,  
GEO. W. PARSONS.